

K. GOLDSCHMIDT & J. WEBER.

DETINNING TIN SCRAP.

APPLICATION FILED AUG. 1, 1906.

1,158,128.

Patented Oct. 26, 1915.

2 SHEETS—SHEET 1.

Fig. 1



Fig. 2



Witnesses:

Paul Wollenberg  
Arthur Schatz

Inventors  
Karl Goldschmidt  
Josef Weber  
by Robert Seippler  
Attorney

K. GOLDSCHMIDT & J. WEBER.

DETINNING TIN SCRAP.

APPLICATION FILED AUG. 1, 1906

1,158,128.

Patented Oct. 26, 1915.

2 SHEETS—SHEET 2.

Fig. 3



Fig. 4



WITNESS

*Chas. J. Clagett*

INVENTORS

*Karl Goldschmidt*  
*Josef Weber*  
BY *John F. Dorn*

ATTORNEY

# UNITED STATES PATENT OFFICE.

KARL GOLDSCHMIDT AND JOSEF WEBER, OF ESSEN-ON-THE-RUHR, GERMANY, ASSIGNEES, BY MESNE ASSIGNMENTS, TO GOLDSCHMIDT DETINNING COMPANY, OF JERSEY CITY, NEW JERSEY, A CORPORATION OF NEW JERSEY.

## DETINNING TIN-SCRAP.

1,158,128.

Specification of Letters Patent. Patented Oct. 26, 1915.

Application filed August 1, 1906. Serial No. 328,793.

To all whom it may concern:

Be it known that we, KARL GOLDSCHMIDT and JOSEF WEBER, subjects of the King of Prussia, German Emperor, and residents of 5 Essen-on-the-Ruhr, Germany, have invented certain new and useful Improvements in Processes of Detinning Tin-Scrap, of which the following is a specification.

All processes of detinning tin clippings, 10 tin cans, or other tin bearing material by means of chlorin that have heretofore been practised, whether they have been carried out with chlorin alone or by chlorin diluted with an inert gas or by the use of chlorin 15 in the presence of an anhydrous liquid present the great drawback that at the points where the reaction takes place, that is, where the stannic chlorid is formed, an excessive temperature is developed, this increase in 20 temperature, however, being an irregular one, the temperature rising to such an extent at certain points in the vessel as to enable the chlorin to affect the iron injuriously, while at other points in the vessel a much 25 lower temperature prevails.

In order to produce a detinned iron that has not been unduly attacked by the chlorin, and in order also that the process as a whole may be carried out in the shortest period 30 of time, it is of the utmost importance that the temperature, though varying from time to time during the detinning period, shall at any given time be as nearly uniform as possible throughout all parts of the apparatus in which the detinning is taking place. 35 This is one of the chief objects of our present invention, and it may be attained by imparting to the particles of the reacting agent, such as chlorin, whether it is used 40 alone or in combination with an inert fluid, in gaseous or liquid form, such a stirring motion as will result in a thorough commingling of the particles in the vessel. By imparting a proper stirring or whirling motion 45 to the fluids or gases in the vessel an immediate equalization of the temperature in the various parts of the apparatus may be obtained and constantly maintained throughout the detinning operation. Such 50 a stirring or whirling motion can be produced by dividing the apparatus or vessel in which the detinning is to take place into two or more chambers, as by means of one

or more partitions, through which chambers the fluids may be constantly circulated in 55 any suitable manner, as for example, by means of a pump by which they may be drawn or forced through each chamber, and if desired, constantly circulated from one chamber into another and back again into 60 that from which they were withdrawn. In this method the stirring or circulating action is produced and takes place entirely within the apparatus in which the detinning takes place. Another method which may 65 be employed consists in drawing off the fluids from one side of the vessel through a pipe outside of the same and returning said fluids to the vessel at the other side of the apparatus, preferably after the gases have 70 been considerably cooled. The equalization of temperature produced by such an agitation or commingling of the gases in the vessel as has just been described is not, however, the only result of the present invention, 75 nor is it the only feature thereof that is of value in the art of detinning.

An important feature of the invention, which extends beyond the mere equalization of the temperature in the different parts of 80 the apparatus, is the rapid cooling of the contents of the apparatus, particularly of the reacting agents contained therein, which cooling is a result of the agitation and commingling of the gases and liquids in contact with a heat-absorbing medium or surface, the best results being obtained in the detinning process when said fluids are circulated in such a manner as to reduce their temperature and that of the other contents 85 of the vessel to a temperature of from 50° to 90° C.

While the importance of cooling the contents of the apparatus during detinning has 95 been generally recognized, it has been found that in detinning on a large scale the use of a water jacket alone does not produce the desired cooling effect. We have found that unless the gases within the vessel are energetically agitated or circulated in contact with a heat-absorbing medium, it is difficult 100 to reduce the temperature of the vessel to the proper extent, as gases in a state of rest and in large masses are such poor conductors of heat that when acted upon in such a state 105 by a cooling agent, such for example as cold

water running over the surface of the apparatus, the reduction of the temperature within the apparatus is very slow. By keeping the gases constantly in motion and circulating them through the vessel in such a manner as to bring fresh particles constantly into contact with the heat-absorbing medium or surface, a very rapid cooling of the gases and other contents of the apparatus results.

This method involves also the additional and great advantage of permitting the thorough detinning of the scrap in a much shorter time than has heretofore been required, and hence a very great economy in the operation of the plant. It is important to bear in mind that as in this process gases are the principal agents used, the number of calories to be absorbed and withdrawn from the apparatus is comparatively large. For example, assuming that a cylindrical vessel made of iron be used, having a diameter of two meters and a height of ten meters, with a total surface of thirty-eight square meters, and that it has a thickness of fifteen millimeters in order to withstand the pressure employed within it, this vessel will ordinarily be filled with about fourteen tons of material containing about 2.35% of tin, and the vessel will contain about 330 kilograms of tin. As the heat of combustion of one kilogram of tin in chlorin is 1078 calories, there will be developed in the vessel an amount of heat represented by 355,740 calories. Now, if we assume that an increase of 40° C. in temperature takes place in the fourteen tons of scrap introduced into the apparatus and in the metal of the apparatus itself, which, if of the above dimensions would weigh about six tons, making a total of twenty tons of iron, the specific heat of which is .105, then this twenty tons of iron will absorb only 84,000 calories of the total heat developed. There would thus remain 271,740 calories which would ordinarily escape into the workroom by radiation from the surface of the apparatus. Now, one square meter of iron will set free at a difference of temperatures of 40° C. about 240 calories per hour by radiation, so that the apparatus above described, which has a surface of thirty-eight square meters, would set free 9120 calories per hour. Hence, about thirty working hours would be required to carry out the process if radiation by the apparatus alone were depended upon to dissipate the heat developed.

The course of the operation will not be much quicker even if the detinning vessel is cooled with water from the outside, for this will only serve to cool those particles of gas which are nearest to the inside wall of the apparatus, and hence the equalization of the temperature within the apparatus will still be very slow.

The cooling of the gases will be much more rapid if those gases are agitated energetically, as before described. If this is done, and the vessel is simultaneously cooled by the outside application of water, the whole process, as has been demonstrated in practice, can be completed in twelve hours instead of thirty. The same result is secured by circulating the gases through an air cooler with a large surface, say one hundred square meters, instead of circulating water around the outside of the apparatus.

In addition to energetically agitating the gases or causing them to circulate through the apparatus, a further means that may be employed for equalizing and reducing the temperature is the introduction of an anhydrous fluid, for example, liquid perchlorid of tin, into the apparatus and into contact with the gases therein. This liquid perchlorid of tin may be introduced at the top of the vessel and caused to flow down, preferably in fine streams, through the gases to the bottom of the vessel, where it may be collected. When introduced in this manner it will circulate oppositely to the gases to be cooled. By employing such an anhydrous heat-absorbing fluid as an auxiliary, the circulating gases readily give up their heat to such anhydrous liquid as well as to the metal of the vessel itself. Thus the anhydrous liquid presents additional heat-absorbing surfaces to the chlorin gas, which, however, must be constantly in a state of agitation and energetically circulating throughout the apparatus, in order to produce the best results. The most intimate contact between the various particles of the gas and the particles of the anhydrous liquid is obtained by circulating the anhydrous fluid through the vessel in fine streams, and preferably in a direction opposite to that in which the gases are moving. An anhydrous heat-absorbing liquid, such as that before described and which may be circulated through the apparatus simultaneously with the chlorin gas, presents the great advantage that it can be more easily cooled, and afterward possesses greater heat-absorbing power, than an equal volume of gas.

In the drawings we have illustrated different types of apparatus for carrying out our improved process.

Figure 1 illustrates a detinning apparatus divided into two compartments by a partition, the view being a vertical section taken in line A—A, Fig. 2; Fig. 2 is a horizontal section of the same, taken in line B—B, Fig. 1; Fig. 3 illustrates in the same manner as in Fig. 1 a similar apparatus showing a modification of the invention; and Fig. 4 is a similar view illustrating said apparatus further modified.

In Figs. 1 and 2 the detinning vessel is divided by a partition *d* into two chambers

- a* and *b*, from the first of which gases flow into the chamber *b*, and from which in turn they are returned to the chamber *a*, at the bottom thereof, and flow upward through said chamber *a*. This circulation of the gases is constantly maintained in any suitable manner, as for example, by means of pumps *v* and *v'*. At the outside of the apparatus cold water is preferably kept constantly circulating by means of a spray or other device *s* over the outer shell or mantle *m* in order to absorb as much as possible of the heat of the shell of the apparatus and of the gases in contact with, or lying close to the inner surface thereof. It will be noted that the more rapid the circulation of the gases within the vessel, the greater will be the cooling effect of the metallic mantle of the apparatus on said gases.
- 10 In Fig. 3, instead of circulating the gases from one chamber to another of the detinning vessel, a pipe *r* is placed outside the apparatus, and the gases are withdrawn from the apparatus at one side through said pipe and returned to the apparatus at the other side thereof. In this case also a pump is preferably employed for the purpose of rapidly circulating the gases through the apparatus and the pipe *r*.
- 15 In order to obtain the best results a system of cooling pipes, such as are shown at *k* in Fig. 4, may be employed to sub-divide the mass or stream and increase the superficial area exposed to the cooling action.
- 20 These pipes may be used either as an auxiliary in the cooling of the gases, or may be used alone, that is, without the simultaneous application of water to the outside or mantle of the vessel.
- 25 In carrying out our improved process we proceed as follows: The apparatus is filled with tin scrap, usually compressed scrap, preferably in bundles, carried in scrap-containers such as *e*, and the apparatus is then closed by suitable means, including a cover *n*, and chlorin introduced under a pressure which may be increased during the detinning, so that the temperature is kept at the desired point. During the introduction of this chlorin gas, which is suitably controlled to produce the desired result, an energetic agitation and circulation of the gas, or of the chlorin gas and the inert gas or gases used in connection therewith, should be begun. Simultaneously the circulation of the anhydrous heat-absorbing fluid, such as liquid perchlorid of tin, may be effected, in order that it may absorb the heat of the chlorin gas while such gas is in rapid motion, this liquid being introduced for example at *p*. By carrying out the process in this manner substantial equality of temperature throughout the vessel is assured, and an energetic circulation of the gases along the cooling surfaces presented by the walls of
- 30 the shell and also by the finely-divided streams of heat-absorbing liquid will result in the rapid cooling of the gases within the vessel, and hence in the carrying out of the whole process in an efficient and economical manner.
- 35 It will be found advantageous not to let the stannic chlorid formed by the process pass through the apparatus with the gases used to bring about the reaction, but to let it drip down, since if it were to pass through the pump the latter would be burdened unnecessarily. This stannic chlorid may be removed by means of a special pump. It may be drawn off during the operation.
- 40 It should be mentioned that it is left entirely to the discretion of the operator whether to use the special cooling means hereinbefore described or to dispense with them and make use only of natural radiation to cool the apparatus and its contents. In every case, however, the energetic agitation or circulation of the gases must be effected in order to avoid a dangerous increase of temperature in various parts of the apparatus and prevent injury of the product.
- 45 By the term "chlorin", as used in the claims, is meant not only chlorin gas alone, but any mixture or combination of chlorin with inert gases or inert liquids, provided that such mixture or combination contains chlorin in sufficient quantity to act as a detinning reagent.
- 50 What we claim is:—
1. The process of detinning tin-scrap which consists in introducing chlorin into a closed apparatus containing the scrap and imparting to the body of gases confined in the apparatus an energetic stirring motion, whereby the temperature is substantially equalized throughout the scrap.
  2. The process of detinning tin-scrap which consists in introducing chlorin into a closed apparatus containing the scrap and imparting to the body of gases confined in the apparatus a stirring motion sufficient to substantially equalize the temperature throughout the scrap, the temperature being maintained at a point below that at which iron is attacked.
  3. The process of detinning tin-scrap which consists in introducing chlorin into a closed apparatus containing the scrap, imparting to the body of gases within the apparatus a stirring motion sufficient to substantially equalize the temperature throughout the scrap, and circulating the gases in contact with a heat-absorbing surface, whereby the temperature of the contents of the tank is maintained at the desired degree.
  4. The process of detinning compressed tin-scrap which consists in introducing chlorin into a closed apparatus containing the compressed scrap and imparting to the body of gases confined in the apparatus an ener-

1. The process of detinning tin-scrap which consists in introducing chlorin into a closed apparatus containing the compressed scrap and imparting to the body of gases confined in the apparatus an energetic stirring motion, whereby the temperature is substantially equalized throughout the scrap.

2. The process of detinning compressed tin-scrap which consists in introducing chlorin into a closed apparatus containing the compressed scrap and imparting to the body of gases confined in the apparatus a stirring motion sufficient to substantially equalize the temperature throughout the scrap, the temperature being maintained at a point below that at which iron is attacked.

3. The process of detinning compressed tin-scrap which consists in introducing chlorin into a closed apparatus containing the compressed scrap, imparting to the body of gases within the apparatus a stirring motion sufficient to substantially equalize the temperature throughout the scrap, and circulating the gases in contact with a heat-absorbing surface, whereby the temperature of the contents of the tank is maintained at the desired degree.

4. The process of detinning tin-scrap which consists in introducing chlorin under increasing pressure into a closed apparatus containing the scrap and imparting to the body of gases confined in the apparatus an energetic stirring motion, whereby the temperature is substantially equalized throughout the scrap.

5. The process of detinning tin-scrap which consists in introducing chlorin into a closed apparatus containing the mass of scrap, imparting to the body of gases within the apparatus a stirring motion sufficient to substantially equalize the temperature throughout the scrap, cooling the chlorin that passes out of the scrap and re-introducing said cooled chlorin into said mass.

6. The process of detinning tin-scrap which consists in introducing chlorin into a closed chamber containing the mass of scrap, cooling the exterior walls of the scrap-containing chamber, imparting to the body of gases within the chamber an energetic stirring motion, and circulating the gases in contact with the cooled walls of the chamber whereby the temperature of the contents of the tank is substantially equalized and maintained at the desired degree.

7. The process of detinning tin-scrap which consists in circulating chlorin through a mass of tin-scrap whereby the temperature is maintained approximately uniform in all parts of the mass and simultaneously

circulating a heat-absorbing fluid in contact with said gas.

8. The process of detinning tin-scrap which consists in circulating chlorin through a mass of tin-scrap whereby the temperature is maintained approximately uniform in all parts of the mass and simultaneously circulating a heat-absorbing anhydrous liquid in contact with said gas. 60

9. The process of detinning tin-scrap which consists in circulating chlorin through a mass of tin-scrap whereby the temperature is maintained approximately uniform in all parts of the mass and simultaneously circulating a heat-absorbing liquid in contact with said gas and in a direction opposite to the flow of said gas. 65

10. The process of detinning tin-scrap which consists in circulating chlorin through a mass of tin-scrap whereby the temperature is maintained approximately uniform in all parts of the mass and simultaneously circulating streams of perchlorid of tin in contact with said gas. 70

11. The process of detinning tin-scrap which consists in circulating chlorin and an inert gas through a mass of tin-scrap whereby the temperature is maintained approximately uniform in all parts of the mass and simultaneously circulating a heat-absorbing fluid in contact with said chlorin. 75

12. The process of detinning tin-scrap which consists in circulating chlorin and an inert gas through a mass of tin-scrap whereby the temperature is maintained approximately uniform in all parts of the mass and simultaneously circulating a heat-absorbing anhydrous liquid in contact with said chlorin. 80

13. The process of detinning tin-scrap which consists in circulating chlorin and an inert gas through a mass of tin-scrap whereby the temperature is maintained approximately uniform in all parts of the mass and simultaneously circulating a heat-absorbing anhydrous liquid in contact with said chlorin. 85

14. The process of detinning tin-scrap which consists in circulating chlorin and an inert gas through a mass of tin-scrap whereby the temperature is maintained approximately uniform in all parts of the mass and simultaneously circulating a heat-absorbing fluid in contact with said chlorin. 90

15. The process of detinning tin-scrap which consists in circulating chlorin and an inert gas through a mass of tin-scrap whereby the temperature is maintained approximately uniform in all parts of the mass and simultaneously circulating a heat-absorbing anhydrous liquid in contact with said chlorin. 95

16. The process of detinning tin-scrap which consists in circulating chlorin and an inert gas through a mass of tin-scrap whereby the temperature is maintained approximately uniform in all parts of the mass and simultaneously circulating fine streams of a heat-absorbing anhydrous liquid through the chlorin in a direction opposite to the flow of said chlorin. 100

17. In witness whereof we have hereunto set our hands in the presence of two witnesses. 105

DR. KARL GOLDSCHMIDT.  
DR. JOSEF WEBER.

Witnesses:

WILLIAM ESSENWEIN,  
ALFR. POHLMAYER.